

# UNITED STATES PATENT OFFICE.

RENÉ CLAVEL, OF BASEL, SWITZERLAND.

## PROCESS FOR PRODUCING FOAM FOR TREATING TEXTILE MATERIALS.

1,234,732.

Specification of Letters Patent. Patented July 31, 1917.

No Drawing.

Application filed April 21, 1916. Serial No. 92,775.

To all whom it may concern:

Be it known that I, Dr. RENÉ CLAVEL, manufacturer, a citizen of the Swiss Republic, and resident of Basel, Switzerland, have 5 invented a new and useful Process for Producing Foam for Treating Textile Materials, of which the following is a full, clear, and exact specification.

Processes are known for treating textiles, 10 such as silk, cotton or wool, either raw or finished, with foam. Originally the foam was produced by boiling solutions of materials adapted to foam and aiding hereby, if desired, the conversion of the solutions into 15 foam by injecting into the solutions air under pressure and in a state of fine division, more recently attempts have been made to work at lower temperatures by producing the foam by diminishing the atmospheric 20 pressure, so that delicate textiles, particularly silk, might be successfully treated.

The processes, therefore, depend upon a supply of heat or steam or upon the action 25 of a vacuum; the high temperature requires a rapid working and the vacuum requires closed vessels.

By the present invention the production 30 of foam is quite independent of the temperature of the foam bath, so that textiles which are sensitive to heat can be treated. The foam is produced by the introduction into the solution or liquid, of air, oxygen or other oxidizing, reducing or indifferent gas under pressure, through finely porous bodies 35 such as tubes or plates of unglazed earthenware, graphite or the like.

The liquid adapted to foam or the solution 40 of a substance of a less foaming tendency, is in this manner saturated with air or other gas and as an emulsion therewith brought into a foaming condition. The foam is of extremely uniform fineness and may be obtained at any temperature from the freezing point to the boiling point of the liquid or 45 solution. The vigorous foaming of the liquid and the extraordinary fineness of the bubbles produce a constant circulation and contact of the bubbles with the fiber, so that constant movement of the textile goods is 50 not necessary, whereby damage of the textile fibers is avoided. Since the production of the foam is independent of the temperature, the bubbles retain substantially their original size, depending only on the size of the 55 pores of the material through which the gas is forced and the pressure at which the fore-

ing occurs. It follows that the fineness of the foam may be varied as desired. The foam made in this manner lasts a long time and can be increased at will; moreover, the 60 whole foam bath is not subject to the oscillations of temperature attendant upon boiling and a predetermined temperature and depth of foam can be maintained easily as may be necessary.

For degumming silk it is advantageous 65 to operate at 75-95° C. The air intimately emulsified in large quantity with the foam favors the degumming by its oxidizing and mechanical action, so that the operation occupies a shorter time than is the case when 70 the foam is produced only by boiling or by the action of a vacuum. At the same time the loss of liquid from the bath is inconsiderable, since the operation is conducted at 75 a temperature below the boiling point.

By emulsifying an oxidizing gas, such as air, oxygen or gas containing oxygen, in the foam, the duration of the de-gumming, owing to the oxidizing action of the gas may 80 be reduced by more than half of the duration of the usual boiling-off process, and contrariwise by emulsifying a reducing gas in the foam the degumming may be prolonged 85 far beyond the usual duration of the operation.

As is known, during the formation of silk thread production of sericin occurs, which is to be referred to the oxidizing action of the air. Probably, during this process only the 90 outer layers form finished sericin, which is separated from the fibroin core by parts gradually less completely oxidized to sericin from the exterior to the interior.

If, for instance, care is taken for abundant access of oxygen during degumming, the complete change of the said incompletely oxidized parts into sericin, and therefore their separation from fibroin, occurs more quickly, that is to say, the de-gumming is 95 of shorter duration.

This effect may also be achieved by adding salts which yield oxygen in nascent condition. Such an addition is free from objection because by emulsifying the nascent gas 105 from the salt, the fibers are not damaged.

For weighting silk the process presents the further advantage that the silk may be treated at a comparatively low temperature with any desired weighting-foam. As is 110 known, for phosphate baths the temperature of the liquid should not exceed 75° C. and

for silicate baths 60° C., since at higher temperatures the silk is strongly attacked by the alkaline action of these salts. The technical improvement is that the silk may be treated sufficiently long in the foam to insure an absolutely uniform saturation and fixing, which is essential for completing the chemical reaction leading to weighting.

The advantages in de-gumming and weighting are: baths of small bulk, immediate formation of foam, much abbreviated duration of the operation, particularly in degumming in which process the silk receives an extraordinary luster. Furthermore, preservation of the goods, as well as a uniform weighting process are secured by the vigorous movement of the finely emulsified bath.

The invention is also particularly useful in degreasing and cleaning raw and finished textiles, for instance in degreasing wool; for it is possible to work with emulsions in the gas foam of solvents for fat such as hydrocarbons, carbon bisulfid, various chlorids of carbon, saturated and unsaturated, or alcoholic substances; the bubbles containing the respective vapor or gas act on the material completely, quickly and with thorough extraction.

The invention is also applicable in dyeing, soaping, degreasing, fixing, mordanting, vat dyeing or developing dyes at any desired temperature, there being used an indifferent, oxidizing, reducing or other chemically acting gas, or mixture thereof, and the textile material being in any form, such as skeins or webs, whether raw, bleached or printed.

What I claim is:

1. A process for producing at any desired temperature foam for treating textile materials, by introducing a gas under pressure into the liquid necessary for the desired treatment through finely porous material, so as to produce foam bubbles with which the gas is emulsified and is in condition to act mechanically on the textile material. 40

2. A process for producing at any desired temperature foam for treating textile materials by introducing a chemically active gas under pressure into the liquid necessary for the desired treatment through finely porous material, so as to produce foam bubbles with which the gas is emulsified and is in condition to act chemically and at the same time mechanically on the textile material. 50

3. A process for producing at any desired temperature foam for treating textile materials by introducing an oxidizing gas under pressure into the liquid necessary for the desired treatment through finely porous material, so as to produce foam bubbles with 60 which the gas is emulsified and is in condition to act in oxidizing manner and at the same time mechanically on the textile material.

In witness whereof I have hereunto signed my name this 20th day of March, 1916, in the presence of two subscribing witnesses.

DR. RENÉ CLAVEL.

Witnesses:

ARNOLD ZUBER,  
AMAND RITTER.